

# UNITED STATES PATENT OFFICE.

ROBERT ABBOTT HADFIELD, OF WESTMINSTER, ALEXANDER GEORGE MCKENZIE JACK, OF BRINCLIFFE, ISAAC BERNARD MILNE, OF TOTLEY, AND ESMOND MORSE, OF SHEFFIELD, ENGLAND.

## MANUFACTURE OF CAPS FOR ARMOR-PIERCING PROJECTILES.

1,363,467.

Specification of Letters Patent. Patented Dec. 28, 1920.

No Drawing.

Application filed July 9, 1919. Serial No. 309,769.

*To all whom it may concern:*

Be it known that we, Sir ROBERT ABBOTT HADFIELD, baronet, F. R. S., ALEXANDER GEORGE MCKENZIE JACK, ISAAC BERNARD MILNE, and ESMOND MORSE, subjects of the King of Great Britain and Ireland, residing, respectively, at the city of Westminster, England, Brincliffe, in county of York, England, Totley, in the county of Derby, England, and Sheffield, in the county of York, England, have invented Improvements in or relating to the Manufacture of Caps for Armor-Piercing Projectiles, of which the following is a specification.

This invention relates to the manufacture or production of caps for armor piercing projectiles or shells of all calibers, particularly of large calibers, say of twelve inches and upward, that shall be better adapted than those heretofore produced to enable such projectiles to perforate thick hard faced armor plates under the special conditions required in naval warfare, namely at long range and therefore at comparatively low velocities, and particularly when striking obliquely at large angles, say of the order of about  $20^{\circ}$  and upward, without becoming broken up, or broken up to such an extent as to interfere with their subsequent desired action.

To enable such a cap to successfully fulfil its required functions, it should be made of metal possessing considerable toughness and tensile strength and capable of being hardened and tempered, and have a rounded or blunt end portion or head capable of striking a hard faced armor plate over a small localized area rather than at a point, without the adjacent part of the cap coming in contact with the plate at the moment of impact, even when striking at a considerable angle. Such front end portion or head should be made of considerable hardness and toughness and be supported by a stiff rear portion so that when the cap is fitted to a projectile, it will, on impact against a hard faced armor plate, cause an initial disintegration of the surface of the plate by reason of the mass of hard metal in its front portion, together with the rigid support of the stiff and tough material in the rear of such hard portion.

In order to produce a cap possessing the

special features or characteristics above set forth, it is made of an alloy steel, for example of nickel chromium steel, of a composition that will admit of its front portion being hardened to a high degree, and of the other required physical and mechanical characteristics being imparted to it by suitable heat treatment. To this end, it may for example be formed of nickel-chromium steel containing from about .50 to .7% of carbon, from about 2 to 4% of nickel and from about 1.5 to 3% of chromium. The cap is formed to the required shape and dimensions, as by casting or forging, or casting and forging, and machining operations and, if desired, it may be annealed in the ordinary way or in any suitable way. The cap may be for example of ordinary conical shape with a rounded front end portion of such dimensions, for example of about one point three inches radius in the case of a cap for a 15" projectile, that when striking an armor plate, only a comparatively small area of such forward end of the cap will come into contact with and disintegrate the face of the plate, even when striking at a large angle, say at  $20^{\circ}$  or more, and so prepare the way for the pointed end portion of the projectile over which the cap is fitted, to successfully attack the plate and enable the projectile to pass successfully therethrough. The front of the cap may be of conical shape if desired and in each case it may be flattened to some extent at its extreme front end over a small area.

The cap after being formed to the required shape is subjected to heat treatment in order to harden and temper it in such a way as to impart to it different degrees of hardness varying say from a ball hardness of from about 600 to 700 at the pointed front end portion or zone through successive rearward zones of about 500, 400 and 300 ball hardness and so that the zones merge gradually one into the other and impart to the cap the required characteristics hereinbefore mentioned.

The degree of hardness corresponding to a ball hardness of 600 and above is herein-after referred to for brevity and distinction as A ball hardness, the degree of ball hardness corresponding to 500 to 600 is 105 hereinafter referred to as B ball hardness,

that corresponding to 400 to 500 as C ball hardness, that corresponding to 300 to 400 as D ball hardness and that below 300 as E ball hardness.

5 Caps of the character above referred to have heretofore been made. For producing such a cap, the cap made of nickel chromium steel, in which the carbon may vary up to .6 to .7%, after being formed to the required 10 shape, has had its front end portion according to some of the methods heretofore adopted, heated to a temperature of about 850° C. after which the cap was dipped while at this temperature in cold water to 15 a zone depth, that is to say, for part only of its axial length, so as to stiffen and harden the cap to the desired degree at different parts thereof, the cap thus treated possessing zones of decreasing ball hardness from 20 its front end, where it has a ball hardness of from 500 to 600 and above, to the rear end portion where it has a ball hardness of from 300 to 200, the cap being thus composed of zones of steel of A, B, C, D, and E degrees 25 of ball hardness.

In this way a cap can be produced having a dead hard front end portion and a stiffened or toughened rear end portion.

The present invention relates to improved 30 methods of hardening and tempering caps of the kind hereinbefore referred to, whereby the special characteristics of hardness, stiffness and toughness now required, can be imparted to the caps in a better manner than 35 heretofore and so that caps having the required characteristics can be produced in a regular or uniform and reliable manner.

For this purpose, a cap, which may advantageously be of nickel chromium steel, 40 such as hereinbefore referred to, after being formed to the desired shape and after having been subjected, it may be, to a preliminary annealing or equivalent heat treatment, is subjected to the following improved heat 45 treatment for hardening and tempering it.

For hardening the cap it is first gradually and uniformly heated to a temperature, say of from about 820 to about 840° C., the higher the hardening element or elements 50 in the steel the lower the temperature used, the cap being finally heated to a practically uniform temperature throughout. The gradual heating of the cap may conveniently be effected in stages or steps in a gas fired furnace having a suitable contrivance for rotating the cap as it is being heated, to insure even heating to a high temperature. It is then quenched by immersing it in a suitable cooling medium to a certain depth 60 and for a convenient time in such a way that by the action of the cooling medium upon the thicker portion of the cap together with or alternately by the action of the air upon the thinner portion, the whole material of the cap is rapidly cooled and so hard-

ened. For instance, the heated cap is, while suitably suspended, for example in a ring-like holder, hardened all over by dipping it point downward to near its base in cold water. The water may then be allowed to 70 gradually run off so that it will first leave the thinner and upper base end of the wall of the cap and gradually recede in a downward direction from the cap, finally leaving the lower solid forward end of the cap. Or 75 the cap, after the water has receded a certain distance, may be taken out of the water, the cap having cooled to such an extent as to retain its hardness. Or the cap may be gradually lifted out of the water by 80 means of a suitable appliance instead of lowering the water level.

By the treatment described, notwithstanding the varying thickness of the metal comprising the cap from its base end to its forward end, the metal can be hardened throughout the whole mass thereof. During this hardening treatment the cap is or may be slowly rotated in the water in order to insure uniformity of hardening. The cap 90 may also be hardened in oil or by other cooling medium, as for example an air blast, at suitably modified temperatures in order to produce the hardness required.

The rate at which the water is run off, or 95 the cap lifted out of the water, can be varied according to the caliber and weight of the cap and to suit different requirements. Satisfactory results have been obtained in the case of a cap for a 13.5" armor piercing projectile and weighing say about 150 pounds, by running off the water to the required depth in about 10 minutes after immersion of the cap. The water is or may be run off through one or more cocks or other valves 100 so that the rate of outflow can be regulated to suit requirement. The rate of outflow of the water, or the rate at which the cap is lifted out of the water, is preferably such that when the cap is sufficiently hardened, 110 it is taken out of the water while it is still hot, but below a temperature of about 200° C., as at this temperature the hardness imparted to the cap will not be affected by the residual heat left in the cap. The cap after 115 removal from the water, is cooled preferably in the air, for which purpose it may be placed on the floor of the shop in which the heat treatment is carried out.

Alternatively, the cap may be immersed 120 in water, preferably running, to a definite depth, or series of definite depths, each for a certain time and then removed from the cooling medium. For example, a 150 lb. cap for a 13.5 inch shell would be immersed substantially to one half its overall length in 125 running water for a period of 9 minutes.

The cap thus hardened throughout its mass is then tempered by heating its rear end portion to impart to the whole cap the 130

required varying degrees of A, B, C, D and E ball hardness. This tempering can be effected in various ways.

According to one way of carrying out the 5 tempering process, the rearward portion of the hardened cap is heated say to a temperature of the order of about 750° C., for a nickel chromium steel such as hereinbefore referred to, while the forward portion of 10 the cap is kept cool or comparatively cool, as for instance by exposing it to the air, the heating being continued for a sufficient time, say for example for about fifteen to twenty minutes in the case of a cap for a 13.5" 15 armor piercing projectile, to reduce the hardness of the cap to the required ball hardnesses while leaving the portion of the cap in front of the point of the shell mainly of A and B ball hardness.

20 For tempering a cap in the manner just described, the cap may advantageously be suspended in a holder base end downward, and immersed to a suitable depth or depths in a bath of molten metal, for example lead, 25 or molten salts, at a temperature of, say for example, the order of about 750° C., and held there until the blue color temper line produced on the exposed surface of the cap reaches a predetermined height, varying for 30 caps of different sizes and to suit different requirements. The base end of the cap may advantageously be immersed to a depth of about 25% of the length of the cap in the molten lead and be held in that position 35 until the blue color temper line reaches a height of about 50% from the base end of the cap, which it will do in about fifteen minutes for a cap suitable for a 13.5" projectile and such as hereinbefore referred to.

40 The cap is then removed from the lead bath, suspended point downward, as in a ring-like holder, and allowed to cool, preferably in the air.

Or the front end portion of the hardened 45 cap, in an inverted position, may be immersed in cold water or other liquid while the other and upper rear portion of the cap is heated, as for example by the application thereto of an annular series of gas flames, 50 to about the temperature mentioned, for a suitable time to temper it to the degree required.

The whole cap may then be allowed to cool in the air.

55 By the means described there can be obtained a hardened and tempered cap having successive zones of A, B, C, D, and E ball hardness extending rearward from its point, there being very considerable volumes of 60 steel of A and B ball hardness and the zones of A, B, C, D, and E ball hardness merging gradually one into the other. Also, by hardening and tempering a cap in the way described, the required varying volumes of 65 steel of A, B, C, D and E ball hardness and

other desirable characteristics can be imparted to the cap in a manner that is under complete control.

The heat treatment temperatures to which the cap is subjected and the depths of immersion of the cap in water and molten lead can be varied to some extent from those mentioned which have been found suitable for the particular steel used in the construction of the cap described.

70 The hardening and tempering treatments hereinbefore described can advantageously be applied to caps of different shapes and made of steel of various kinds.

75 What we claim is:—

1. A process for the manufacture of a cap for an armor piercing projectile from alloy steel capable of being hardened and tempered, said process consisting in heating the cap to a substantially uniform temperature 85 and quenching the required length of it in a suitable cooling medium so that the whole of the cap is rapidly cooled and hardened, then heating its rear end portion while its point is kept cool or comparatively cool, to 90 temper the cap and finally cooling the cap.

2. A process for the manufacture of a cap for an armor piercing projectile, said process consisting in heating a cap made of nickel chromium steel to a substantially uniform 95 temperature and quenching the required length of it in water so that the whole of the cap is rapidly cooled and hardened, then heating its rear end portion while its point is kept substantially cool, to temper the cap 100 in the required manner and finally cooling the cap.

3. In the process as claimed in claim 2, finally cooling the cap in air after heating it for tempering.

4. In the process as claimed in claim 2, heating the cap to a temperature of the order of from about 820 to 840° C. preparatory to quenching it.

5. In the process as claimed in claim 1, 110 hardening the cap by immersing it in a cooling liquid from its point to some desired extent of its length.

6. In the process as claimed in claim 1, 115 hardening the cap all over by immersing it, point downward, in a cooling liquid nearly to its base and then gradually reducing the influence of the cooling medium thereon by varying the level of the liquid relatively to the cap.

7. In the process as claimed in claim 1, 120 hardening the cap all over by immersing it, point downward, in a cooling liquid nearly to its base end and then gradually withdrawing it from the influence of the 125 cooling liquid by running off the liquid.

8. In the process as claimed in claim 1, 130 hardening a cap made of nickel chromium steel of substantially the composition herein set forth, by heating it to a temperature of

- the order of about 820 to 840° C. and immersing it point downward in water nearly to its base and then gradually withdrawing it from the cooling influence of the water.
- 5 9. A process of tempering a cap that has been hardened all over, said process consisting in heating the rear end portion of the cap, for a suitable time, to a suitable tempering temperature while its front end portion
- 10 is exposed to a cooling medium and afterward slowly cooling the said rear end portion of the cap.
10. In the process as claimed in claim 1, tempering a cap that has been hardened,
- 15 by supporting the cap point upward and immersing a suitable length of its rear end portion in molten material at a suitable temperature.
11. In the process as claimed in claim 1,
- 20 tempering a cap that has been hardened, by supporting the cap point upward and immersing a suitable length of its rear end portion in molten metal at a suitable temperature.
- 25 12. In the process as claimed in claim 1,
- tempering a cap that has been hardened, by inserting the cap base end downward for approximately 25% of its overall length, in a bath of molten lead at a suitable temperature while exposing its front end portion to a cooling medium and removing the cap from the molten bath when the hardness of each portion of the whole cap has been reduced to the requisite degree.
13. In the process as claimed in claim 1, tempering a cap that has been hardened, by inserting the cap base end downward for approximately 25% of its overall length in a bath of molten lead at a suitable temperature, while exposing its front end portion to the air, removing the cap from the molten bath when the hardness of each portion of the whole cap has been reduced to the requisite degree and cooling the cap in air.

Signed at London, England, this fourth 45  
day of June, 1919.

ROBERT ABBOTT HADFIELD.

ALEXANDER GEORGE MCKENZIE JACK.

ISAAC BERNARD MILNE.

ESMOND MORSE.